

# United States Patent Office

2,894,910

Patented July 14, 1959

1

2,894,910

## WATER-IN-OIL EMULSION LUBRICANTS

Charles E. Francis, Martinez, and Norman Bulman, Berkeley, Calif., assignors to Shell Development Company, New York, N.Y., a corporation of Delaware

No Drawing. Application July 23, 1956  
Serial No. 599,329

5 Claims. (Cl. 252—42.7)

This invention relates to improved emulsion lubricants and hydraulic fluids. More particularly it pertains to water-in-oil emulsion lubricants especially useful for slow speed diesel engines and as fire-resistant hydraulic fluids which possess good lubricating properties and which are stable, non-corrosive and wear-resistant.

Although it is known in the art that certain emulsions are useful as coolants and lubricants in metal working operations and as rust and corrosion inhibitors, their use as engine lubricants and as hydraulic fluids has been limited. Under engine operating conditions, emulsions generally lack desired lubricity, cause wear and corrosion.

Fluid compositions for use in many hydraulic systems should be fire-resistant, non-corrosive, thermally stable and resistant to oxidation. Hydraulic fluids such as mineral oils or other organic fluids such as castor oil, esters of carboxylic acids, organic phosphates, glycols and their derivatives, silicone polymers, chlorinated or fluorinated organic materials as well as aqueous solutions, lack one or more desired properties which such fluids should possess. Thus, mineral oils are highly flammable, castor oil results in sludge and gum formation, esters of carboxylic acids cause swelling of rubber, the organic phosphates and the glycols are corrosive, the halogen-containing materials tend to hydrolyze, while the silicone compounds lack lubricity and present a health hazard.

It is an object of this invention to provide an emulsion lubricant and fire resistant hydraulic fluid having good lubricating properties. Another object is to provide a composition which is a satisfactory lubricant for low speed diesel engines and hydraulic equipment, which is stable, fire-resistant, resistant to deterioration, inhibits corrosion and does not cause wear. Still another object of this invention is to provide an emulsion lubricant and fire-resistant hydraulic fluid of good lubricating quality even when subjected to various adverse conditions of temperature, loads and speeds as encountered in various diesel engines operating on high sulfur fuels or in certain hydraulic systems.

These and other objects are accomplished in accordance with this invention by providing a composition comprising a water-in-oil emulsion in which the water phase is from 20% to 45% and the oil phase is from 55% to 80% of the emulsion, said emulsion containing a combination of minor amounts each of two essential additives one of which is an oil-soluble polyvalent metal phenate and the other is an oil-soluble high molecular weight alkane-polyol. They may be obtained as polymeric compounds by substantially completely hydrolyzing a copolymer of a long chain alpha olefinic hydrocarbon (normal or branched-chain) containing a terminal  $-\text{CH}=\text{CH}_2$  group, and containing at least 10 carbon atoms, and a vinyl ester of a lower fatty acid having up to five carbon atoms, such as vinyl acetate, vinyl propionate, vinyl isobutyrate, or vinyl isovalerate. The final product is a macromolecular organic compound containing essentially a plurality of recurring alkyl-1,2-ethylene and hydroxy-1,2-ethylene units joined together in a chain-like manner,

2

wherein the alkyl radicals contain at least 8 carbon atoms. There may be a minor proportion of alkanoyloxy-1,2-ethylene (from unhydrolyzed ester groups) units as essentially the only other polar-containing group. The ratio of the non-acidic oxygen containing units (hydroxyl- and alkanoyloxy-) 1,2-ethylene to the alkyl-1,2-ethylene units is from about 1 to about 5 and the average molecular weight of the final product is from about 4,000 to about 50,000. The non-acidic oxygen-containing polar groups present in the final product are predominantly hydroxyl, being at least 80% hydroxyl, preferably at least 90% or as high as 99% of the non-acidic oxygen-containing polar groups.

The oil-soluble phenates which are effective in combination with the higher alkane polyols water-in-oil emulsions of this invention include those described in United States Patents 2,197,833, 2,228,654, 2,280,419, 2,344,988, 2,361,804, 2,410,652, 2,501,991, 2,501,992 and 2,610,982. Specifically, they can be either simple phenates, such as metal alkylphenates (Ca cetylphenate), polar substituted simple phenates (Ca or Zn alkyl salicylates) or polyphenates, such as where a plurality of the simple phenates are condensed at positions ortho and/or para to the phenolic hydroxy group through alkylidene (e.g. methylene) radicals or other suitable divalent non-metallic radicals, such as sulfur or selenium. Although various metal phenates are contemplated in the practice of the invention including mono- and polyvalent metal phenates, such as the alkali, alkaline earth and heavy metal phenates, of which the preferred ones are the polyvalent metal phenates of the metals of group II of the periodic table and having an atomic number of from 12 to 56, especially the alkaline earth metals within that group of metals. Illustrative compounds are: Na, K, Li, Ca, Ba, Sr, Mg, Zn, Al, Cd, Ni, Fe, Co cetylphenate, dibutylphenate,  $\text{C}_{14}\text{—C}_{18}$  alkyl salicylate, waxylphenate, cyclohexylphenate, octylthiophenate, cetylthiophenate as well as the above metal salts of the condensation product of alkyl phenol with formaldehyde, acetaldehyde, furfuraldehyde or benzaldehyde, e.g., Ca, Ba, or Mg salts of octyl phenol-formaldehyde condensation product ranging in molecular weight of from 400 to 1,100.

The oil-soluble phenates are effective in the emulsions in amounts of from about 0.01% to about 10%, the amount preferably being from about 0.1% to about 5% by weight.

In the polymeric material broadly described it is believed that the polar-containing and non-polar units are substantially uniformly distributed throughout the length of the hydrocarbon chain in accordance with the respective molecular proportions of the olefin and ester monomers utilized in the preparation with some randomness from exact regularity. Furthermore, even where two polar containing ethylene units are bound directly, the polar groups in general are attached to nonadjacent carbon atoms.

The alpha olefins suitable to form the copolymers include olefins having a single terminal ethylenic group and containing from 10 to 40 carbon atoms and preferably from 12 to 30 carbon atoms such as  $\alpha$ -decene,  $\alpha$ -hexadecene,  $\alpha$ -tetradecene,  $\alpha$ -pentadecene,  $\alpha$ -heptadecene,  $\alpha$ -octadecene,  $\alpha$ -nonadecene,  $\alpha$ -eicosene,  $\alpha$ -docosene,  $\alpha$ -triacontene, and mixtures thereof. Mixtures of  $\alpha$ -olefins containing from 12 to 20, and preferably 16 to 18 carbon atoms obtained by pyrolysis of paraffin waxes, are particularly suitable and represent a readily available economic material.

The unsaturated esters which are useful to make the copolymer are exemplified by vinyl esters of lower saturated fatty acids, such as vinyl acetate, vinyl propionate, vinyl butyrate, vinyl isovalerate, and mixtures thereof.

Normally, these reactants are copolymerized in the

presence of a catalyst. Catalysts which are suitable for the copolymerization include various organic peroxides, such as aliphatic, aromatic, heterocyclic, and alicyclic peroxides such as diethyl peroxide, tertiary butyl hydroperoxide, dibenzoyl peroxide, dimethylthienyl peroxide, dicyclohexyl peroxide, dilauroyl peroxide, di-tert-butyl peroxide, and urea peroxide. These specific peroxides are mentioned by way of nonlimiting examples of suitable organic peroxides.

The identity and proportion of catalyst selected and the temperature employed in the copolymerization can be varied to produce products having different molecular weights as desired. Thus, if one desires lower molecular weight products, one might select a higher reaction temperature, such as of the order of 150° C. to 300° C., and select a catalyst that has a satisfactory decomposition rate within that range of temperature. When a higher molecular weight product is desired, a lower temperature range may be used, such as 50° C. to 150° C., and a catalyst having a satisfactory decomposition rate within that range may be selected. In general, it is preferred to employ temperatures within the range of 80° C. to 200° C. and catalysts which are effective within that range.

The polymerization may be conducted in the presence or absence of air. In most cases, however, it has been found desirable to conduct the polymerization in the absence of air, e.g., in the presence of an inert gas such as nitrogen. Atmospheric, reduced, or superatmospheric pressure may be employed.

At the end of the polymerization, unreacted monomer is removed, usually suitably by distillation.

The conversion of the ester groups to hydroxyl groups can be accomplished by hydrolysis or alcoholysis. Hydrolysis or alcoholysis can be accomplished by the methods described in U.S. Patent 2,421,971. Hydrolysis may be by saponification, with aqueous alkali, such as sodium hydroxide, or by alcoholysis reaction wherein the copolymer is treated with a lower water-soluble alkanol, e.g. methyl, ethyl or isopropyl alcohol, or mixture of a lower alkanol and a suitable base catalyst, such as sodium ethoxide.

After the saponification or alcoholysis, the mixture is treated to remove materials other than the desired product, such as by distillation to remove volatile materials and by water-soluble salt impurities, such as sodium acetate. It is particularly important to remove water-soluble salts in order to obtain copolymers which can be used as additives for fuel oils without forming undesirable haze.

The following examples are given as illustrative of suitable products and their preparation.

#### EXAMPLE I

About 21.8 moles of C<sub>16</sub>-C<sub>18</sub>  $\alpha$ -olefins and 54.4 moles of undistilled vinyl acetate were heated to about 140° C.

with stirring and about 0.3% w. of di-tert-butyl peroxide was added and the mixture heated for about 5 hours. An amount of vinyl acetate equal to that charged was added to the mixture at such a rate that the vinyl acetate/olefin ratio in the unreacted vinyl acetate to olefin was around 2.5. After 5 hours of heating the reaction mixture was topped to remove unreacted vinyl acetate and peroxide decomposition products. About 97% of the polymerizable olefins were converted to polymer.

The polymer was alcoholized by refluxing it for about two hours with a mixture of methanol and aromatic solvent containing a small amount of sodium methoxide. To this was added a mixture of aromatic solvent and water and the entire mixture was shaken, allowed to separate into layers at 50-60° C. and the upper phase was removed. The material was then heated to 125° C. to remove residual methanol, methyl acetate and water. The aromatic solvent can be removed by stripping at a temperature of 180° C. at 1 mm. The ratio of vinyl acetate to olefin in the polymer was around 4.85 and the molecular weight ranged around 30,000 to 35,000.

#### EXAMPLE IA

2.5 moles of vinyl acetate and 1 mole of a mixture of C<sub>16</sub> to C<sub>18</sub> alpha olefins, predominantly C<sub>18</sub> olefins, and 1% tertiary butyl peroxide were placed in a stainless steel bomb and the air replaced with nitrogen. The bomb was heated to 115° C. until there was about 90% conversion. The product was topped at 185° C. at 1 mm. Hg pressure.

The polymer product was then mixed with methanol and sodium methylate so as to effect a 95% conversion of the acetate groups to hydroxyl groups. This was accomplished by adding 10 parts of methanol, 35 parts of isopropyl alcohol and 1 part of sodium methylate per 50 parts of the copolymer and neutralizing with stirring for 8 hours at 70° C. Sodium acetate was then removed by washing twice with 1 part of a 33% isopropyl alcohol-water mixture. After settling, the lower layer was drained off and all low boiling components stripped off at a temperature of 110° C. at 90 mm. Hg. The resulting copolymer was a sticky yellow solid.

#### Analysis:

|    |                                                                                                  |      |
|----|--------------------------------------------------------------------------------------------------|------|
| 45 | Mol ratio of acetate plus alcohol groups to olefin C <sub>14</sub> -C <sub>16</sub> alkyl groups | 5/1  |
|    | Mol wt.                                                                                          | 2700 |
|    | Mol ratio of hydroxyl to acetate groups                                                          | 19/1 |

Following essentially the procedure of Example I, other products were prepared as Examples II through XXI in accordance with the following tabulation showing the polymerization catalyst, polymerization temperature, ratio of vinyl ester to olefin used and ratio in the product, degree of hydrolysis of the ester groups and average molecular weight.

| Example | Catalyst                 | Temperature, °C. | Vinyl Acetate/ $\alpha$ -Olefin Ratio in Polymer | Vinyl Acetate/ $\alpha$ -Olefin Ratio in Polymer | Degree of Hydrolysis | Mol Wt. <sup>1</sup> |
|---------|--------------------------|------------------|--------------------------------------------------|--------------------------------------------------|----------------------|----------------------|
| II      | ditertiarybutyl peroxide | 115              | 2.5/1(C <sub>16</sub> -C <sub>18</sub> Olefin)   | 5                                                | 92                   | 27,000               |
| III     | do                       | 115              | 1.9/1(C <sub>15</sub> -C <sub>18</sub> Olefin)   | 2.6                                              | 95                   | 11,000               |
| IV      | do                       | 115              | 1/1(C <sub>16</sub> -C <sub>18</sub> Olefin)     | 2                                                | 95                   | 8,000                |
| V       | do                       | 130              | 2.5/1(C <sub>16</sub> -C <sub>18</sub> Olefin)   | 4.9                                              | 92                   | 20,000               |
| VI      | do                       | 140              | do                                               | 5                                                | 95                   | 20,000               |
| VII     | do                       | 140              | 4.0/1(C <sub>16</sub> -C <sub>18</sub> Olefin)   | 4.9                                              | 90                   | 30,000               |
| VIII    | benzoyl peroxide         | 80               | 1.6/1(octadecene)                                | 3.6                                              | 95                   | 16,500               |
| IX      | do                       | 80               | 2/1(octadecene)                                  | 4.06                                             | 97                   | 20,000               |
| X       | do                       | 110              | do                                               | 3.4                                              | 88                   | 8,330                |
| XI      | do                       | 80               | do                                               | 1.52                                             | 95                   | 5,120                |
| XII     | do                       | 80               | do                                               | 1.72                                             | 95                   | 5,710                |
| XIII    | do                       | 80               | 2.5/1(octadecene)                                | 4.1                                              | 95                   | 20,100               |
| XIV     | do                       | 80               | 2/1(octadecene)                                  | 3.89                                             | 97                   | 14,200               |
| XV      | do                       | 115              | 3/1(octadecene)                                  | 4.1                                              | 90                   | 11,000               |
| XVI     | do                       | 80               | 2/1(dodecene)                                    | 2.6                                              | 90                   | 8,000                |
| XVII    | do                       | 80               | 2/1(hexadecene)                                  | 3.1                                              | 90                   | 8,000                |
| XVIII   | do                       | 60               | do                                               | 2.14                                             | 90                   | 16,400               |
| XIX     | do                       | 80               | 2/1(vinylbutyrate/ $\alpha$ -octadecene)         | 2.1                                              | 90                   | 8,000                |
| XX      | do                       | 80               | 1/1.2(octadecene)                                | 1                                                | 95                   | 8,000                |
| XXI     | do                       | 80               | 1/1.2(hexadecene)                                | 1                                                | 95                   | 8,000                |

<sup>1</sup> Mol wt. determined by light scattering technique described in Chem. Res., vol. 40, p 139 (1948).

The polymers are effective when used in amounts of from about 1% to about 10% by weight and preferably from about 1.5% to about 5% by weight, based on the total composition.

The aqueous phase of the water-in-oil emulsion should range from about 20% to about 45% and preferably from about 30% to about 40% by weight of the emulsion. The oil phase can vary from about 55% to about 80% and preferably from about 60% to about 70% of the emulsion. The oil may be entirely a hydrocarbon oil of wide viscosity range, e.g., from less than 50 SUS at 100° F. to 150 SUS at 210° F.

Oils of this type can be obtained from various crudes such as paraffinic, naphthenic or mixed base crudes; refined oils in the lubricating oil viscosity range are preferred. On the other hand, the hydrocarbon oil may be blended with fixed oils such as castor oil, lard oil and the like, and/or with synthetic lubricant such as polymerized olefins, organic esters of organic and inorganic acids, e.g., di-2-ethylhexyl sebacate, dioctyl phthalate, trioctyl phosphate; polymeric tetra-hydrofuran, polyalkyl silicone polymer, e.g., dimethyl silicone polymer and the like. Where mixtures or blends are used the hydrocarbon oil such as a mineral lubricating oil is always present in the predominant amount such as from about 60% to about 95% of the oil blend. A straight mineral lubricating oil, having a viscosity index of at least 50 and ranging in viscosity at 100° F. of from 75 to 200 SUS, is usually preferred.

and the alkane polyol, while constantly stirring the mixture. Heating the emulsion during or after it is prepared is not necessary. If desired, the emulsion can be homogenized to insure a homogeneous composition.

- 5 A composition (A) of this invention was prepared by slowly adding 40% water into a vessel containing 60% of a refined mineral oil of 150 SUS viscosity at 100° F., and containing 1.5% polymer of Example I and 4% of Ca salt of octyl phenol-formaldehyde condensation product, while constantly stirring the mixture. The entire mixture was transferred to a homogenizer where it was agitated for about 5 minutes until a homogeneous water-in-oil emulsion was formed. Compositions (B), (C) and (D) were prepared in a similar manner except that 10 the products of Example IA, VII and VIII were used in place of the alkane polyol of Composition (A).

15 Other examples of this invention include a water-in-oil emulsion containing from 1% to 5% of polymers of Example I, III, V, VII or VIII and from 1% to 10% of calcium or barium (neutral or basic) cetyl phenate alkylsalicylate and the like.

20 The outstanding properties of hydraulic fluids of this invention with respect to stability and fire-resistance are shown in Table I. The stability test is determined by 25 determining the amount of separation of free oil, cream and water at both room temperature and 140° F. from a 100 ml. test sample. The fire-resistance was determined by the pipe cleaner test described in Lubrication Engineering, March-April 1955, pages 86-87.

Table I.—Emulsion stability test

| Composition                                                                                                                                                | Days | Room Temperature             |                                | Percent Water Separation (cc.) | Days | 140° F. Percent Oil Separation (cc.) | Percent Cream Separation (cc.) | Percent Water Separation (cc.) |
|------------------------------------------------------------------------------------------------------------------------------------------------------------|------|------------------------------|--------------------------------|--------------------------------|------|--------------------------------------|--------------------------------|--------------------------------|
|                                                                                                                                                            |      | Percent Oil Separation (cc.) | Percent Cream Separation (cc.) |                                |      |                                      |                                |                                |
| A                                                                                                                                                          | 62   | 2                            | 0                              | Trace                          | 13   | 5                                    | 0                              | 1                              |
| B                                                                                                                                                          | 62   | 2                            | 0                              | Trace                          | 13   | 5                                    | 0                              | 1                              |
| C                                                                                                                                                          | 62   | 2                            | 0                              | Trace                          | 13   | 5                                    | 0                              | 1                              |
| D                                                                                                                                                          | 62   | 2                            | 0                              | Trace                          | 13   | 5                                    | 0                              | 1                              |
| Water/oil emulsion (40/60) containing 1.5% Ex. VII additive                                                                                                | 62   | 50                           | 0                              | 10                             | 3    | 8                                    | 10                             | 3                              |
| Water/oil emulsion (40/60) containing 4% Ca salt of octyl phenol formaldehyde condensation product                                                         | (1)  | (1)                          | (1)                            | (1)                            | (1)  | (1)                                  | (1)                            | (1)                            |
| Water/oil emulsion (40/60) containing 1.5% additive of Ex. VII and 8% Ca petroleum sulfonate                                                               | 13   | Trace                        | 30                             | 0                              | 2    | 1                                    | 10                             | Trace                          |
| Water/oil emulsion (40/60) containing 1.5% additive of Ex. VII and 1% glycerol monooleate                                                                  | 37   | 1                            | 38                             | Trace                          | 7    | 1                                    | 48                             | 12                             |
| Water/oil emulsion (40/60) containing 1.5% additive of Ex. VII and 5% octadecylamine                                                                       | 24   | 2                            | 29                             | Trace                          | 7    | 1                                    | 32                             | 2                              |
| Water/oil emulsion (40/60) containing 1% alkyl phenoxyethylene ethanol (Igepal DM-710 made by Antara Chemicals Division of General Aniline and Film Corp.) | 5    | (2)                          | (2)                            | (2)                            | 5    | 1                                    | 70                             | 3                              |
| Water/oil emulsion (40/60) containing copolymer of vinyl pyridine/lauryl methacrylate                                                                      | (1)  | (1)                          | (1)                            | (1)                            | (1)  | (1)                                  | (1)                            | (1)                            |
| Water/oil emulsion (40/60) containing copolymer of vinyl pyrrolidone/lauryl methacrylate                                                                   | (1)  | (1)                          | (1)                            | (1)                            | (1)  | (1)                                  | (1)                            | (1)                            |
| Water/oil emulsion (40/60) containing copolymer of lauryl methacrylate/diethylamine ethyl methacrylate                                                     | (1)  | (1)                          | (1)                            | (1)                            | (1)  | (1)                                  | (1)                            | (1)                            |

<sup>1</sup> Complete phase separation.

<sup>2</sup> Complete phase.

Compositions of this invention can be modified by addition thereto of minor amounts (0.01-12%) of optional additives such as corrosion inhibitors, stabilizers, anti-wear agents, and the like, but which do not interfere with the essential additives of this invention and which are compatible with the emulsion without materially altering the stability and other properties of the emulsion. Included among such materials are inorganic and organic salts such as water-soluble polyvalent metal salts such as calcium, barium or magnesium nitrite, nitrate, sulfate, chloride, chromate, formate, acetate and the like.

Compositions of this invention are readily prepared. No special equipment or technique is necessary in the preparation of them. A preferred method is to add the required amount of water to the oil containing the phenate

In the pipe cleaner test, Compositions A through D passed over 50 cycles while mineral oil or mineral oil containing 4% of Ca petroleum sulfonates and/or Ca salt of octylphenol-formaldehyde condensation product 65 ignited after about 5 cycles.

Compositions of this invention are particularly suitable for use in diesel engines, in die casting machines, in permanent mold machines in steel mill equipment such as coke pushers, pipe coupling tighteners, combustion control mechanisms, plastic molding presses and glass blowing machines and the like.

We claim as our invention.

1. A lubricant and hydraulic fluid consisting essentially of a water-in-oil emulsion in which the water phase constitutes from about 30 to about 40% of the emulsion and

the oil phase constitutes from about 70% to about 60% of the emulsion, said emulsion containing from about 1 to about 10% by weight of hydrolyzed copolymer of a hydrocarbon  $\alpha$ -olefin containing from 10 to 40 carbon atoms and a vinyl ester of a lower fatty acid having up to 5 carbon atoms in the mol ratio of from 1/1 to 1/5, respectively and having a molecular weight of from 4,000 to 50,000 and from about 0.01% to about 10% of an oil soluble polyvalent metal  $C_{8-18}$  alkyl phenate of the metal of group II of the periodic table having an atomic number of from 12 to 56.

2. The composition of claim 1, wherein the metal phenate is an alkaline earth metal  $C_{8-18}$  alkyl phenate and the hydrolyzed copolymer is a copolymer of an  $\alpha$ -olefin containing from 12 to 30 carbon atoms and a vinyl ester of a lower fatty acid of up to 5 carbon atoms.

3. The composition of claim 1, wherein the polyvalent metal phenate is calcium  $C_{8-18}$  alkyl phenate and the copolymer is a hydrolyzed copolymer of a  $C_{16-18}$   $\alpha$ -olefin and vinyl acetate.

4. A lubricant and hydraulic fluid consisting essentially of a water-in-oil emulsion in which the water phase constitutes about 40% of the emulsion and the oil phase is 60% of the emulsion, said emulsion containing about 0.1 to about 5% by weight calcium salt of octylphenol-formaldehyde condensation product and from about 1.5 to about 5% by weight of a hydrolyzed copolymer of a  $C_{16-18}$  hydrocarbon  $\alpha$ -olefin and vinyl acetate in the mol ratio of from 1/1 to 1/5, respectively and having a molecular weight of from 4,000 to 50,000.

5. The composition of claim 4, wherein the olefin and vinyl acetate constituents in the polymer are in the ratio of from 1:2 to 1:4, respectively.

15

References Cited in the file of this patent

UNITED STATES PATENTS

|           |                    |       |               |
|-----------|--------------------|-------|---------------|
| 2,421,971 | Sperati            | ----- | June 10, 1947 |
| 2,551,643 | Seger et al        | ----- | May 8, 1951   |
| 2,744,870 | Stillebroer et al. | ----- | May 8, 1956   |
| 2,800,453 | Bondi              | ----- | July 23, 1957 |

20